

## UNITED STATES PATENT OFFICE

LAUBI I. L. DURCHMAN, OF PETERSBURG, VIRGINIA

## METHOD FOR MANUFACTURING HIGH-GRADE ALPHA CELLULOSE

No Drawing.

Application filed May 8, 1929. Serial No. 361,545.

My invention relates to a new and useful method for manufacturing high-grade alpha-cellulose suitable for making explosives, rayon, lacquers, etc., from unbleached easy 5 bleaching sulphate or soda-cellulose, independent of what kind of wood has been used in the pulping process. This method as described below can wholly or partly be used for that same purpose to treat sulphite or 10 any kind in chemical way pulped suitable fibrous material.

The unbleached sulphate cellulose contains a large number of incrusting substances thus as lignins, pentosans, fats, waxes and rosins 15 which give the pulp a certain color variable from pale yellow to dark brown. The ordinary kraft pulp contains about 75-85% of alphacellulose and the rest is beta and gamma cellulose known by the collective 20 name hemicelluloses. To make the pulp easier for bleaching it has to be digested in a certain known way with a certain amount of alkaline solution and at a certain pressure for a certain time. Thus digested pulp contains between 80-90% alphacellulose. But 25 still the incrusting substances and the color are very resistant against every bleaching agent so the pulp has to be given a certain treatment prior to the bleaching to avoid 30 an excess of bleaching solution which would increase the bleaching costs and decrease the percentage of alphacellulose.

The present invention comprehends the preliminary treatment before bleaching the cellulose, the bleaching of the cellulose with an alkaline bleaching solution, the treatment of thus bleached pulp with white liquor, (sulphate or soda) containing as main part NaOH and the final treatment with oxalic 40 acid.

As above mentioned the cellulose has after it has been washed, screened and thickened to be given a treatment prior to the bleaching to dissolve and remove organic matters 45 which resist against the bleaching agents.

This treatment has to be carried out in an open tank using a mixture of from 2% to 5% sodium hydroxide (NaOH) or with corresponding amount of so called white liquor and from 1% to 3% sodium sulphite 50 (Na<sub>2</sub>SO<sub>3</sub>) based on the dry weight of the cellulose for 5 to 6 hours. Better results are obtained if this operation is done in a digester under certain conditions of pressure and time. Satisfactory results are obtained 55 by cooking from 4 to 6 hours at a pressure of from 20 to 60 pounds. This cooking action dissolves a great proportion of the ligneous and resinous compounds and forms 60 water-soluble organic compounds which can be thus removed.

After being thoroughly washed and thickened the cellulose is to be bleached with an alkaline bleaching solution which contains from 1-3% of sodium sulphite based on the 65 bleaching powder which is used to make up the bleaching solution. The temperature after 2-3 hours bleaching can be raised to about 40-45 degrees C. The presence of alkali prevents oxidation and too quick bleaching action and decomposes certain ligneous and resinous compounds, so that the loss is only from 2-4%, while by using a calcium hypochlorite solution the losses are from 4-8%, and sometimes higher. It is preferable to use two stage bleaching adding at first about  $\frac{2}{3}$  of the necessary amount of bleaching solution and after the chlorine is exhausted and the pulp thoroughly washed to add the second part or last  $\frac{1}{3}$  of the solution. The principle of this kind of bleaching is to chlorinate the liquors and other incrusting matters in the first stage and to oxidize the coloring matters in the second stage. The pulp has then to be washed thoroughly, thickened and centrifuged to highest possible dryness before adding the usual 80 cooking or white liquor containing Na<sub>2</sub>S, Ma<sub>2</sub>Co<sub>3</sub> and as main part NaOH. The total amount of alkali in this so-called white 85 liquor is about 10% of the weight of the pulp. The pulp is then washed again to remove the alkali and the bleaching liquor. The final product is a white cellulose which is 90

liquor is usually 120-180 gr. per liter and as effective NaOH 100-140 gr. per liter.

This treatment with alkali effects the dissolving of the less resistant substances known as beta and gamma celluloses and depending upon the amount of alphacellulose in the pulp after the bleaching and upon the strength of the alkaline solution used and of the time and temperature of the treatment, certain grades of high alphacellulose ranging from 90-100% can be obtained. By adding the alkaline (white) liquor to the bleached pulp it becomes a yellow greenish color which mostly disappears by adding a very small amount of acetic, lactic, or oxalic acid. If the color should not disappear the cellulose has to be treated with a small amount of bleaching solution for a short time. This treatment will restore and increase the whiteness of the pulp. The white liquor such as used in the soda and sulphate pulp mills has to be well settled or filtered so it will not contain any sludge which would increase the ash and iron in the pulp. After the treatment is finished the cellulose has to be centrifuged to highest dryness so that the highest possible amount of used alkaline (white) liquor can be recovered and used without any treatment for cooking of the wood chips. The strong wash-water can be used for the first cooking treatment prior to the bleaching. The total recovered amount of white liquor is from 80-90%. For the manufacture of rayon, lacquers, explosives, films, etc., a low ash and iron content is required so the cellulose after the alkaline treatment has to be given a treatment to remove the calcium and to dissolve the iron compounds. I have discovered that oxalic acid is a very suitable agent to use because it dissolves the iron and precipitates the calcium compounds which are in or around the fiber cells, not completely, but to a certain extent. An absolutely complete precipitation of the calcium compounds is not possible without using a great excess of oxalic acid and thereby decreasing the alphacellulose percentage through oxidation by the strong organic acid solution because the organic matters in the fibers prevent the influence of the acid to react completely with the calcium compounds. The amount of oxalic acid necessary to precipitate the calcium compound is dependent upon the amount of ash the pulp contains after the strong alkaline treatment, but 6-8% oxalic acid based on the dry weight of the pulp gives an excess of oxalic acid which is necessary to reach the desirable precipitation of calcium compounds to calcium oxalates. About 80-90% of the used oxalic acid can be recovered. The cellulose is then thoroughly washed and dried on a Fourdrinier or Sargent drying machine.

My invention may be briefly illustrated by a flow sheet as follows:

*Flow sheet*

Easy bleaching pulp (sulphate 90-94% alphacellulose). 70

Washed, screened and thickened.

I Digesting in open tank.  
With NaOH (2-5%) + Na<sub>2</sub>SO<sub>3</sub> (1-3%) based on air dry weight of the pulp.

↓  
Centrifuging and washing } Strong liquor to the wash pans. 75  
Weak liquor to the sewer.

II Bleaching, washing and centrifuging.

III Treatment with white liquor containing from 10-14% NaOH. 80  
Strong liquor to chip digestion.  
Weak liquor to 1st treatment.

↓  
Centrifuging and washing.

IV Treatment with 6-8% oxalic acid based on air dry weight of the pulp.

↓  
Centrifuging and washing. → Oxalic acid for reuse.

V Drying of the 97-99% alphacellulose.

Having thus fully described my said invention, what I claim as new and desire to secure by Letters Patent, is:

1. The process of treating chemical wood pulp to convert incrusting substances into water-soluble compounds comprising treating the pulp for a period of four to six hours at 20 to 60 pounds pressure with a solution containing 2% to 5% NaOH and 1% to 3% Na<sub>2</sub>SO<sub>3</sub>. 95

2. The process of treating cellulose material to remove incrusting substances therefrom which comprises treating such cellulose material for a period of four to six hours with a mixture of from 2% to 5% sodium hydroxide and 1% to 3% sodium sulphite at a pressure of from 20 to 60 pounds. 100

3. The process of treating chemical wood pulp to convert incrusting substances into water-soluble compounds comprising treating the pulp for a period of four to six hours at 20 to 60 pounds pressure with a solution containing 2% to 5% NaOH and 1% to 3% Na<sub>2</sub>SO<sub>3</sub>, bleaching, and thereafter treating the bleached pulp at room temperature for three to five hours with white liquor to effect removal of incrusting substances for obtaining a high grade alphacellulose. 110

4. The process of treating chemical wood pulp to convert incrusting substances into water-soluble compounds comprising treating the pulp for a period of four to six hours at 20 to 60 pounds pressure with a solution containing 2% to 5% NaOH and 1% to 3% Na<sub>2</sub>SO<sub>3</sub>, bleaching, thereafter treating the bleached pulp at room temperature for three to five hours with white liquor to effect removal of incrusting substances for obtaining a high grade alphacellulose, washing, and treating the pulp with an organic acid to neutralize residual alkali and to extract other residual and coloring impurities; thereby re- 125

storing the whiteness of pulp discolored by treatment with white liquor.

5. The process of treating chemical wood pulp to convert incrusting substances into water-soluble compounds comprising treating the pulp for a period of four to six hours at 20 to 60 pounds pressure with a solution containing 2% to 5% NaOH and 1% to 3% Na<sub>2</sub>SO<sub>3</sub>, bleaching, thereafter treating the 10 bleached pulp at room temperature for three to five hours with white liquor to effect removal of incrusting substances for obtaining a high grade alphacellulose, treating the pulp with oxalic acid to precipitate the calcium compounds and to dissolve the iron compounds, and washing the pulp to remove the iron and calcium compounds.

In testimony whereof I affix my signature.  
LAURI I. L. DURCHMAN.

20

25

30

35

40

45

50

55

60

65